

# United States Patent Office.

ISAAC E. CRAIG, OF CAMDEN, OHIO.

*Letters Patent No. 74,314, dated February 11, 1868; antedated January 30, 1868.*

## IMPROVEMENT IN THE MANUFACTURE OF SHEET IRON.

The Schedule referred to in these Letters Patent and making part of the same.

TO ALL WHOM IT MAY CONCERN:

Be it known that I, ISAAC E. CRAIG, of Camden, in the county of Preble, and State of Ohio, have discovered a new and improved Method of Manufacturing Sheet Iron; and do hereby declare the following is a full and exact description thereof.

The nature of my discovery consists in so softening the iron to be rolled into sheets, by alloying tin therewith, that after it is rolled into sheets it does not need to pass through an annealing process, to give it the required softness and flexibility for use in the arts.

To enable others skilled in the art to make use of my invention, I will proceed to describe the method of operating the same.

The iron used may be of any of the different kinds of pig which are known as "mill-iron," or used in mills for the purpose of making refined iron. The tin is the ordinary bar or block-tin of commerce. The tin may be alloyed with the pig-metal at any time when it is in a molten state, but the inventor believes the best method is to introduce the tin into the molten iron in a bloomery or knobbling fire, when it is almost ready to stiffen up and be worked into the "loup." No great importance attaches, however, to the exact time of introducing the tin, as the alloy, when once formed, is not liable to separate. The tin should be cut up into small pieces before being cast into the molten metal, and distributed as equally as possible through the metal, and afterward carefully stirred. In the boiling or reverberatory furnace, the alloying of the metals may be effected in the same way, but the quality of the manufactured iron will be as much inferior to that made in the bloomery as ordinary boiled iron is to charcoal-iron; or the alloy may be made in a large crucible, containing steel in a molten state, as in the crucibles for the manufacture of Bessemer steel, after the steel is produced, and while still melted. In this case, however, care should be had to cover the surface of the steel with powdered charcoal, to prevent the loss of tin by oxidation before the metals are alloyed.

When the metals are ready for rolling, the process of "louping" or "balling up" not differing from the common one, they are rolled in the ordinary manner, and polished, by the process understood, by rollers; polishing being an effect of friction, from passing the sheets, in packs, at a low heat, between either soft or chilled sheet rolls, when, after shearing, they are ready for the "bundler."

The proportion of tin necessary to be used varies with different grades of pig-metal; being, as a general rule, from five to ten per cent. of the quantity of iron, five per cent. being enough for good soft iron, a larger proportion being required for inferior grades. As a trial proportion, the discoverer recommends seven or eight per cent. of tin. If, with this proportion, the produced sheets should be softer than needed, a less percentage of tin may afterward be used; if not soft enough, a larger proportion of tin is needed; the softness, without annealing, as in the enclosed sample, affording the manufacturer a ready means of determining, after a few trials, the proper proportion for any grade of pig-metal, it being possible that the proportion of tin may sometimes pass out of the above-mentioned limits.

What I claim as my invention, and desire to secure by Letters Patent, is—

Softening of iron intended to be rolled into sheets, by the alloying of tin therewith.

ISAAC E. CRAIG.

Witnesses:

J. M. SHEAVER,  
E. C. SHEAVER.